

## UNITED STATES PATENT OFFICE.

WARREN F. BLEECKER, OF BOULDER, COLORADO.

## IMPERVIOUS CHEMICAL MATERIAL AND METHOD OF ITS PRODUCTION.

No Drawing.

Application filed January 13, 1923. Serial No. 612,514.

My invention relates to impervious and chemically-resistant material and the method of its production and its principal object resides in providing a material suitable for use in making pipe linings, conduits and machine parts, which is impervious to liquids and gases and proof against the corrosive action of acids and other chemicals and which owing to a high degree of tensile strength and elasticity, is particularly adapted as a substitute for other materials heretofore used for similar purposes.

The material is of a composite character and its principal and essential constituent elements are sulfur and a chemically-resistant body-forming substance, and it is a further object of the invention, to provide in the production of material of a molten mixture of the above stated substances, certain means and treatments which prevent the growth of large sulfur crystals and promote the formation of small crystals desirably to or near the point of being amorphous, and which cause the particles and molecules of the ingredients to be compacted so as to form a dense and substantially non-porous body devoid of voids and gas holes.

The means above referred to may consist of a substance which if added to the mixture opposes the formation of large crystals by re-action with the molten sulfur, and the treatments productive of a similar result, may consist in any action which decreases the cooling period of the molten mixture, after it has been formed into the desired shape, to a point of solidification, or in any action productive of an intermolecular movement, and it should be understood that any two or more of the above mentioned expedients may be combined for co-operative action, if so desired.

Among the substances best adapted to promote the formation of small crystals by re-action with the sulfur, as hereinbefore explained, are those capable of supplying hydrocarbons at the required working temperatures.

Coal tar pitch or charcoal meet every requirement and other kinds of pitch having the desired percentage of readily available hydrocarbons may be used to advantage.

The methods for decreasing the cooling period of the molten sulfur mixture and effecting an intermolecular movement in the same, may consist in rapidly cooling the mass by

artificial means, in agitating or stirring the mass to a point of solidification, or in the proper application of pressure during the cooling period, each action having for its purpose to separately or in conjunction with others, prevent the formation of large sulfur crystals and the occurrence of voids due to gasification of the molten sulfur, as hereinbefore explained.

An important function of the body giving chemically-resistant substance intermixed with the sulfur, is to give to the material the necessary tensile strength, increase its elastic limits and decrease its co-efficient of expansion, and among the materials best suited for the purpose may be mentioned artificial graphite, sand, coke and pulverized slate, it being evident that the physical characteristics of the material may be varied by the use of different substances of the above type, and that their selection is for this reason, governed to a large extent by the particular use or action for which the material or the article produced therefrom is intended and designed.

Inasmuch as artificial graphite is most suitable for the greater number of uses for which the material is intended, the following description will be limited to its employment with the understanding that other materials of the above described character may be substituted therefor in the same or different proportions according to varying requirements and within the scope of the present invention.

An efficient method of reducing the solidification period of the molten sulfur mixture consists in rapidly cooling a surface with which the fluid mass engages, preferably while the mass is under pressure, which causes the fluid matter to be compacted and restrained under gradual and progressive solidification.

In the production of pipe linings, the above described action may be obtained by introducing the mixture in a molten condition into a pipe which is heated above the melting temperature and imparting to the pipe in a substantially horizontal position, a revolving motion about its longitudinal axis which forces the fluid material to the interior surface of the pipe under the influence of centrifugal force. While the pipe is thus revolved, its outer surface is cooled by any suitable means such as a continuous application of cold water or other cooling fluid, with the

result that the fluid matter is rapidly solidified progressively from its outer strata which engages with the surface of the pipe, inwardly, while at the same time the inner portion 5 of the liquid mass is continuously fed to the cooling surface by the centrifugal pressure.

A microscopic examination of a lining thus produced, reveals a total absence of large 10 crystals and a compact arrangement of molecules without noticeable voids or crevices. In fact, the crystals are so small as to approach an amorphous condition and the formation is so dense as to be substantially non-porous.

15 While the above method of forming conduits and pipe-linings of limited thickness is both practical and effectual, it will be evident that other means may be employed to obtain a similar result and that in the production 20 of machine parts of different character which do not permit of the employment of centrifugal force or of rapid cooling in the aforesaid manner, other methods must be resorted to to obtain the required movement of 25 the molecules in the fluid mixture and oppose the tendency of forming large crystals.

An effectual method of producing the desired result in the production of articles of 30 different forms and proportions consists in subjecting the liquid mass to an agitative or stirring action until it has cooled to a point of solidification. During this action artificial cooling means may be applied to the matrix in which the material is formed, it 35 being understood that in this method as well as in the first described process, rapid cooling of the material from one side to another is highly advantageous.

Different methods of subjecting the material 40 to pressure while it cools in the required form may be availed of where the employment of centrifugal force is not feasible or practical, and conduits or pipe-linings may if so desired, be formed by ramming or pressing 45 the fluid matter into a space between the pipe and a therewith concentric core and cooling the exterior surface thereof as before, or by pouring the molten mixture into the pipe with a header of sufficient size to 50 forcibly feed the liquid mass to the interior surface of the pipe during the cooling action.

The pressure to which the material is subjected, should always be sufficient to cause the liquid portion of the material to enter into the 55 pores of that which is already partially solidified by the cooling action upon the surface of the mold and that in the formation of pipe linings and conduits, it is advisable that their thickness should be maintained within certain 60 definite limits on account of the poor conductivity of the sulfur mixture.

In all of the above described actions, the exact nature of the mixture is of secondary consideration provided that it contains an 65 adequate percentage of sulfur, it being evi-

dent that the character and proportions of the other ingredients are subject to variation in accordance with different requirements.

It is, however, as stated hereinbefore, within the scope of the present invention to add to a mixture of sulfur and a finely divided body-giving substance, other ingredients which aid in adapting it for the purpose of producing an impervious and chemically-resistant material of the desired degree of density, tensile 70 strength and elasticity, and to form the material from said mixtures by any one or more of the above described actions, and I desire it understood that my invention as herein disclosed, includes the composition of the chemically-resistant sulfur mixture as well as the methods of forming it into an impervious material, and that either expedient may be employed separately or in conjunction with the other, as may be desirable to expediently 75 and expeditiously produce a material impervious to liquids and gases, having the desired degree of resistance to the corrosive action of acids and other chemicals.

A hydrocarbonaceous substance such as 80 pitch, if added to the sulfur mixture not only aids in opposing the formation of sulfur crystals, but also prevents the occurrence of voids and the development of cracks by temperature variations, increases the modulus of 85 elasticity and otherwise improves the character of the material and generally enhances its adaptability for the purposes for which it is intended.

In order to produce the desired chemical 90 combination of the sulfur and the hydrocarbons, the mixture is heated to a point where chemical action takes place, which under ordinary conditions is indicated by frothing and by the evolution of poisonous gases.

The temperature has been found to be above the melting point of sulfur and although at the present time no definite percentage of hydrocarbons can be given, principally owing to the differences in the materials adapted for their provision, it appears that less than thirty per cent of the sulfur content of the mixture produces satisfactory results.

The hydrocarbons by chemically combining with the sulfur, reduce the size of the sulfur crystals and at the same time permit of admitting to the mixture more hydrocarbons for further chemical combination or mere addition, it being understood that aside 115 from the results obtained by chemical re-action, the size of the sulfur crystals will be restricted in inverse ratio to the percentage of hydrocarbons in the mixture.

In reducing the period of solidification of 120 the molten sulfur mixture by rapid artificial cooling, a ratio may be maintained between the temperature of the cooling medium, the time of application and the percentage of hydrocarbons in the mixture, it being apparent 130

that owing to their similar functions in the production of the material, the factors should be proportioned so as to co-operate without waste of time, labor or material, toward the 5 production of a material of the required character.

While in the foregoing description, hydrocarbons have been mentioned as best adapted to produce the desired action upon the sulfur, 10 it should be remembered that as mentioned hereinbefore, other materials having similar functions, may be employed within the spirit of my invention.

What I claim and desire to secure by Letters Patent is:

1. An impervious chemically-resistant ma-

terial having in intermixture with artificial graphite, sulfur and solid hydrocarbons chemically combined.

2. An impervious chemically-resistant material consisting of artificial graphite intermixed with a chemical combination of sulfur and a hydrocarbon having a high melting point.

3. An impervious chemically-resistant material consisting of artificial graphite intermixed with a chemical combination of sulfur and pitch.

In testimony whereof I have affixed my signature.

WARREN F. BLEECKER.